

June 23, 1936.

L. A. CLARKE

2,045,321

SOLVENT EXTRACTION OF HYDROCARBON OIL

Filed April 19, 1932



LOUIS A. CLARKE  
INVENTOR

BY *R. J. Dearborn*  
HIS ATTORNEY

## UNITED STATES PATENT OFFICE

2,045,321

## SOLVENT EXTRACTION OF HYDRO-CARBON OIL

Louis A. Clarke, Fishkill, N. Y., assignor to The Texas Company, New York, N. Y., a corporation of Delaware

Application April 19, 1932, Serial No. 606,110

5 Claims. (Cl. 196—13)

This invention relates to a process for extracting hydrocarbon lubricating oils with a selective solvent, and more particularly relates to a process of effecting the removal of those hydrocarbons which tend to lower the viscosity index of a hydrocarbon lubricating oil. The invention is directed especially to the process of extracting hydrocarbon lubricating oils with methyl acetate.

It has been found that the hydrocarbons which tend to lower the viscosity index of a hydrocarbon lubricating oil are soluble in methyl acetate, and by extracting the oil with methyl acetate these hydrocarbons may be removed by the solvent and separated from the remaining oil, thereby producing a lubricating oil having a high viscosity index, a low sulphur content, and having extreme resistance to oxidation; such refined oils are also characterized by showing low carbon residue when tested according to the Conradson method.

The invention also contemplates continuously and countercurrently extracting lubricating oil with the solvent, methyl acetate.

It is well known that petroleum products generally contain four groups or types of hydrocarbons, namely, paraffins, naphthenes, aromatics and unsaturates. Of these, the paraffins are the least reactive and the aromatics and unsaturates the most reactive, the naphthenes occupying intermediate positions in the ascending order of reactivity.

This ascending order of reactivity is believed also to be paralleled by the degrees of polarity of the four enumerated types of hydrocarbons. The paraffins are considered to be strictly non-polar while naphthenes, aromatics and unsaturates are polar. It has been demonstrated that the paraffins or non-polar hydrocarbons are characterized by having high viscosity indices while the polar bodies which may include the naphthenes, aromatics and unsaturates have low viscosity indices. It is known that the solubilities in polar solvents of the four groups of hydrocarbons vary directly as their reactivities and their polarities, with the paraffins being the least soluble and the aromatics and unsaturates the most soluble.

Prior to my invention, it was thought that extremely polar solvents, among which may be enumerated sulphur dioxide, liquid ammonia and

liquid carbon dioxide, were necessary for the extensive extractions which must be made in order to permit of the isolation of the paraffin hydrocarbons. Of these solvents, sulphur dioxide has most commonly found favor. Its application, however, has certain drawbacks. Sulphur dioxide is under normal conditions a gaseous material and in order to bring it into the liquid form and to maintain it in that condition, low temperatures and high pressures are necessary. Installations for extracting hydrocarbon oils with liquid sulphur dioxide therefore involve costly apparatus for liquefying the solvent, high pressure vessels for carrying out the extractions at low temperatures and complex distillation equipment for liberating and recovering the sulphur dioxide dissolved in the products of the extraction.

Now I have found that methyl acetate, which is a liquid under normal conditions of temperature and pressure, may be used for the extraction of polar hydrocarbons from hydrocarbon mixtures which function it performs much more efficiently and successfully than even sulphur dioxide. I have applied this characteristic of methyl acetate to the preparation of lubricating oils which after treatment therewith are substantially paraffinic in character and which are characterized by their high viscosity indices, are low in sulphur, resistant to oxidation and yield low Conradson carbon residues. The extraction with methyl acetate may be carried out at normal temperatures and pressures; this is a distinct advantage. Complex equipment and solvent purifying systems are not necessary in its application. Its chemical stability is of such a high order that special materials are not necessary in the construction of the apparatus in which it is used. Its boiling point of 57.5° C. is of such a low order of magnitude as to permit its ready separation from both the extracted oil and from the extract which it has dissolved from the oil. It is not, however, so volatile as to necessitate a special vapor recovery system. Experience has shown that by using a closed system, the solvent loss by this method of refining is exceedingly small.

For a better understanding of my invention, reference may be had to the accompanying drawing which sets forth a flow sheet of a countercurrent treating system which may be used with advantage in the application of my invention.

The numeral 9 indicates a storage tank for unextracted oil. This is connected by line 11 which is fitted with a control valve 10, to a mixing chamber 12 wherein the unextracted oil is 5 agitated with partly spent methyl acetate from a subsequent extraction step. This chamber is in turn connected by line 13 with a settling chamber 14 which may advantageously be of greater diameter than the mixing chamber. 10 Herein the mixture of partly extracted oil and completely spent methyl acetate having in solution low viscosity index or polar bodies separated from the oil is allowed to stratify. The partly extracted oil is drawn off from an upper 15 point in the settling chamber 14 through line 16, which is controlled by valve 15, and is introduced into mixing chamber 21. It is there agitated with fresh methyl acetate which is supplied from the methyl acetate storage tank 59. 20 through the line 19 which in turn is controlled by valve 20. The mixture of extracted oil and partly spent methyl acetate having in solution further quantities of polar bodies extracted from the oil is then passed through line 22 into settling chamber 23. This settling chamber is similar in construction to settling chamber 14. Stratification of the mixture is allowed to take place in this vessel, the supernatant extracted oil containing in solution a small amount of methyl 25 acetate being drawn off through line 25 which is controlled by valve 24. The partly spent methyl acetate containing in solution polar bodies is passed through line 26 controlled by valve 27 into mixing chamber 12. 30 The treated oil containing in solution a small quantity of methyl acetate is then circulated by means of pump 28 through the coils 29 of the heater 30. The oil having been heated is discharged from the heater 30 and is then permitted to expand through valve 32 into a flash 35 tower 33, wherein substantially all of the solvent is distilled off from the treated oil. The vapors of methyl acetate pass out through line 34 fitted with valve 35 which connects the uppermost point in the tower 33 to the inlet 54 of the condenser coils 55. The bottom of tower 33 is connected by line 37 controlled by valve 36 with a cooler 38 from which the cool treated oil is drawn off through line 39 into the treated oil 40 storage tank 40.

The completely spent methyl acetate having in solution the polar or low viscosity index bodies extracted from the treated oil is drawn off from the bottom of settling chamber 14 through line 18 controlled by valve 17 and passes to the suction side of pump 41. This pump circulates the solution of low viscosity index bodies in methyl acetate through the coils 42 of heater 43 from which it passes through line 44 to expansion 45 valve 45 where it is expanded into flash tower 46. The evolved vapors of methyl acetate are drawn off from the top of tower 46 through line 47 controlled by valve 48 into the inlet 54 of condenser coils 55. The bottom of the tower 46 is fitted with a drawoff line 49 controlled by valve 50 through which the extract freed from methyl acetate is passed into cooler 51 and from which it passes to the extract storage tank 53 by way of line 52. 55

The combined methyl acetate vapors from flash towers 33 and 46 pass through inlet line 54 into the coils 55 of condenser 56 wherein condensation takes place. The liquid methyl acetate is drawn off through line 58 controlled by 60

valve 57 into the methyl acetate storage tank 59.

In the preferred manner of practicing the invention with the apparatus illustrated in the drawing, a suitable lubricating oil of low viscosity index and which may have been subjected to treatment with sulphuric acid is passed into the mixing chamber 12 at a temperature of approximately 70° F. wherein it is thoroughly agitated with partly spent methyl acetate from a subsequent step in the treating operation. Simultaneously an equal volume of methyl acetate is introduced at the other end of the treating circuit, namely, mixing chamber 21. The unextracted paraffin oil is agitated in mixing chamber 12 with partly spent methyl acetate from a subsequent step in the treating operation. The mixture of partly extracted oil and spent methyl acetate saturated with extract is then passed into settling chamber 14 wherein stratification of the oil and saturated methyl acetate is allowed to take place. The supernatant partly extracted oil is then passed into mixing chamber 21 wherein it is agitated with fresh methyl acetate, the volume of which is equal to the volume of unextracted oil. 15 20 25

The mixture of completely extracted oil and partly spent methyl acetate is then passed into the final settling chamber 23 wherein stratification is allowed to take place. The lower layer of partly spent methyl acetate having in solution the polar or low viscosity index bodies from the treated oil is then passed to the aforementioned mixing chamber 12 while the supernatant treated oil, comprising approximately 65% of the unextracted oil introduced into the system and containing a small amount of methyl acetate in solution, is then pumped through the coils 29 of heater 30 wherein it is raised to a temperature of approximately 220° F. and a pressure of 40 about 20 lbs. per square inch. 35

The extracted oil having in solution a small quantity of methyl acetate is then expanded through valve 32 into stripping tower 33 to approximately atmospheric pressure which results 45 in the vaporization of the methyl acetate. These vapors are passed out of the stripping tower through the vapor line 34 while the residual treated oil is drawn off from the bottom of the tower through line 37 to a cooler in which its 50 temperature is reduced to approximately 90° F.

Concurrently, the spent methyl acetate having in solution a volume of low viscosity index bodies, approximately 35% of the original unextracted oil, is pumped through the coils 42 of 55 heater 43 wherein the temperature is raised to 220° F. and to a pressure of approximately 25 lbs. per sq. in. It is then expanded through valve 45 into stripping tower 46 to a pressure of approximately atmospheric. The vapors of methyl acetate are drawn off through vapor line 47 while the extract which composes the bottoms is drawn off through line 50 into cooler 51 wherein the temperature is reduced to approximately 80° F. The cooled extract is passed to extract storage tank 53. 60 65

The vapors of methyl acetate obtained from stripping towers 33 and 46 are brought together into the inlet 54 of condenser coils 55 wherein their temperature is reduced to 60° F. which effects substantially complete condensation. The condensed methyl acetate is then drawn off through line 58 into methyl acetate storage tank 59. 70 75

A heavy red paraffin oil having the following tests

|                                         |         |
|-----------------------------------------|---------|
| Gravity, A. P. I.                       | 24.9    |
| Flash, Cleveland open                   | 440° F. |
| Fire                                    | 505° F. |
| Pour                                    | 40° F.  |
| Viscosity, Saybolt universal at 100° F. | 375     |
| 130°                                    | 164     |
| 210°                                    | 54      |
| 10 Sulphur                              | 0.37%   |
| Iodine value                            | 20.4    |
| Viscosity index                         | 77.8    |
| Carbon residue                          | 0.19    |

15 was submitted to extraction with methyl acetate whereby a quantity of low viscosity index bodies to the amount of 35% of the original unextracted oil was separated. The tests of the treated or extracted oil as well as of the extract are given 20 herewith:

|                                        | Extracted oil | Extract |
|----------------------------------------|---------------|---------|
| 25 Gravity A. P. I.                    | 30.4          | 22.3    |
| Flash, Cleveland open                  | 455° F.       | 445° F. |
| Fire                                   | 525° F.       | 495° F. |
| Pour                                   | 55° F.        | 20° F.  |
| Viscosity Saybolt universal at 100° F. | 271           | 472     |
| 130°                                   | 134           | 200     |
| 210°                                   | 52            | 56      |
| 30 Sulphur                             | 0.09%         | 0.49%   |
| Iodine value                           | 10.2          | 26.6    |
| Viscosity index                        | 108.4         | 58.0    |
| Carbon residue                         | 0.09          | 0.55    |

35 It is to be understood that the figures quoted above serve merely to illustrate a typical operation of the process and accordingly may vary. The constitution of the oil to be extracted as well as the characteristics and yield of the extracted oil desired, will determine the relative volumes of 40 unextracted oil and methyl acetate introduced into the system as well as the temperatures necessary for stripping the methyl acetate from the extracted oil and from the extract.

In the foregoing specific example the extraction 45 was carried out at a temperature of about 70° F. or normal room temperature and such temperatures are preferred in extracting with methyl acetate since high yields of high viscosity index oil may be secured. However, other temperatures of extraction may be employed ranging from above the pour point of the oil being treated to about 130° F. depending upon the character of oil and the extent of extraction required. Obviously, the temperature in any event should be sufficient to maintain the oil during extraction 55 completely liquid.

The apparatus shown and described is especially suited for extracting hydrocarbon oils with methyl acetate. While I have thus specifically described my invention and cited an example to illustrate it, the same is not to be construed as limiting the invention, and only such limitations should be imposed as are indicated in the appended claims.

65 I claim:

1. The method of producing a lubricating oil of high viscosity index from a lubricating oil fraction containing hydrocarbons of both high and low viscosity index which comprises mixing and agitating the lubricating oil fraction with methyl acetate at about normal room temperature, allowing the mixture to remain undisturbed

to effect stratification, drawing off the supernatant layer of treated oil and a relatively small amount of methyl acetate and separating said methyl acetate from the treated oil by distillation.

5 2. The continuous method of refining mineral oil containing hydrocarbons of both high and low viscosity index with methyl acetate to produce lubricating oil of a high viscosity index, low in sulphur and Conradson carbon content and 10 resistant to oxidation which comprises alternately mixing together and then separating flowing bodies of the oil and the methyl acetate at about normal room temperature, the relatively saturated methyl acetate coming into contact with 15 relatively fresh oil while the relatively finished oil comes into contact with fresh methyl acetate, and maintaining the bodies of oil and methyl acetate at a temperature of about 70° F. during 20 the treatment.

3. The continuous method of refining mineral oil containing hydrocarbons of both high and low viscosity index with methyl acetate to produce lubricating oil of a high viscosity index, low in sulphur and Conradson carbon content and 25 resistant to oxidation which comprises alternately mixing together and then separating flowing bodies of the oil and the methyl acetate, the relatively saturated acetate coming into contact with 30 relatively fresh oil while the relatively finished oil comes into contact with fresh acetate, and maintaining the bodies of the oil and methyl acetate at about normal room temperature, while the relatively finished oil comes into contact with fresh methyl acetate, forming one portion of liquid composed of methyl acetate and dissolved material extracted from the oil and another portion composed of refined oil and a relatively small amount of methyl acetate, separately heating 35 said liquid portions to a temperature at which 40 the methyl acetate is vaporized, condensing the evolved vapors of methyl acetate, separately cooling the remaining treated oil and extract, and returning the separated condensed methyl acetate 45 for extracting fresh oil.

4. The process of preparing a lubricating oil of high viscosity index from a lubricating oil fraction containing hydrocarbons of both high and low viscosity index by extraction with methyl 50 acetate which comprises alternately mixing together and then separating flowing bodies of the lubricating oil fraction and methyl acetate at about normal room temperature, the relatively saturated methyl acetate coming into contact 55 with relatively fresh oil while the relatively finished oil comes into contact with fresh solvent methyl acetate.

5. The process of preparing lubricating oil of high viscosity index from a lubricating oil fraction containing hydrocarbons of both high and low viscosity index by solvent extraction which 60 comprises mixing and agitating said fraction with a solvent liquid comprising methyl acetate, while maintaining the mixture at about normal room temperature forming a dissolved phase comprising low viscosity index constituents of the oil dissolved in methyl acetate and an undissolved phase comprising high viscosity index constituents of the oil mixed with a relatively small amount of methyl acetate, separating the two phases, and 65 removing the solvent liquid therefrom.

70 LOUIS A. CLARKE.